

## UNITED STATES PATENT OFFICE

1,980,801

## ALLOY

Henry Edwin Holbrook, Irvington, N. J., assignor  
to The H. A. Wilson Company, Newark, N. J.,  
a corporation of New Jersey

No Drawing. Application June 16, 1933,  
Serial No. 676,092

2 Claims. (Cl. 75—1)

This invention relates to alloys and has reference particularly to alloys for use in making contacts or sparking points for electrical apparatus.

5 In the manufacture of such contacts, it is of the utmost importance that the metal composition employed be such as will minimize corrosion and pitting of the contacting surfaces. Another consideration of primary importance is 10 a high degree of uniformity throughout a quantity of the contacts prepared in accordance with procedure which is largely automatic.

I have found that these desirable characteristics are attained in a high degree in contacts 15 which are well adapted for use in electrical apparatus when an alloy is employed containing osmium as a major alloying element. Preferably the osmium is present in the alloy in an amount ranging between 50% and 90%, the proportion 20 which I have found best being about 66% or two parts out of three by weight. The remainder of the alloy is preferably made up of one of the metals rhodium, platinum, palladium, iridium and ruthenium.

25 The best results in the practice of my invention are attained in an alloy consisting mainly of osmium, and secondarily of rhodium. Pref-

erably these two constituents are present in the relation of 66% osmium and 34% rhodium by weight.

This composition has been productive of the best results which I have attained, but it must be understood that there may be some variation without substantial sacrifice in the operating results. The dominant feature of the invention resides in the use of osmium as the major element of the alloy. The proportion of the osmium should be at least 50% and it may be carried as high as 90%, though, as above stated, 66% is the amount which has been found to be best. Much of the remainder of the alloy, preferably all of it, consists of one of the metals, rhodium, 65 platinum, palladium, iridium and ruthenium, and the alloy of osmium and rhodium in the relation of two to one by weight has been found to be best.

I claim:

1. An alloy containing osmium in an amount 75 between 50% and 90%, the remainder being rhodium.

2. An alloy composed of commercial osmium and commercial rhodium, the osmium comprising about 66% and the rhodium about 34% by weight. 80

HENRY EDWIN HOLBROOK.

30

85

35

90

40

95

45

100

50

105

55

110